

## UNITED STATES PATENT OFFICE.

FRED W. WAGNER, OF PITTSBURGH, PENNSYLVANIA, ASSIGNOR TO JONES & LAUGH-LIN STEEL CORPORATION, OF PITTSBURGH, PENNSYLVANIA, A CORPORATION OF PENNSYLVANIA.

## METHOD OF TREATING WASTE OF BENZOL RECOVERY.

No Drawing.

Application filed April 25, 1923. Serial No. 634,604.

*To all whom it may concern:*

Be it known that I, FRED W. WAGNER, residing at Pittsburgh, in the county of Allegheny and State of Pennsylvania, a citizen 5 of the United States, have invented or discovered certain new and useful Improvements in Methods of Treating Waste of Benzol Recovery, of which improvements the following is a specification.

10 My invention relates to the disposal of by-products of coke distillation.

In the recovery of by-products in the industry alluded to, the coke-oven gas is scrubbed, that is to say, is under suitable 15 and predetermined conditions of pressure and temperature, brought into intimate mixture with an absorbent menstruum, ordinarily a heavy oil of the paraffin series, derived from, or perhaps consisting of, petroleum. By such mixture the vapors of certain normally non-gaseous substances, present in the gas, are absorbed by the menstruum, and the denuded gas passes on, to 20 serve such purposes as may at the particular place and under the particular circumstances, be found expedient. The menstruum with its burden of absorbed substances is distilled, ordinarily in a steam still, at a temperature of 150° C., and a distillate is thus obtained which is known as 25 light oil. The menstruum remains in the still, and may be taken and used again. Or the steps of absorption and distillation may be performed in continuity upon a continuously circulating stream of menstruum.

From the light oil so obtained benzol, toluol and the xylols (solvent naphthas) are derived by fractionation. The residue 30 from this fractionation is essentially the absorbent oil which in relatively small quantities passes over with the distillate in the initial distillation.

The fractions of benzol, toluol, and the xylols require first to be washed, before 35 there are marketable. To this end they are treated, each by itself, with sulphuric acid, for the separation of impurities, then they are neutralized, and then subjected again to distillation. The distillate is of marketable 40 purity. The residue in the still is, at the present time waste. All that I have up to this point described is known to the art. My invention deals with this waste, and beginning with it I shall describe my invention.

This residue consists essentially and chiefly of coumarone (compounds of the C<sub>8</sub>H<sub>6</sub>O type), and with it lesser quantities of naphthalene, oils of high boiling point, sulphonated products, but no substantial 60 quantity of the absorbent oil with which the coke-oven gas initially was caused to mingle.

However, I preferably modify somewhat the operation which as ordinarily conducted I have outlined. Beginning with the light 65 oil, instead of fractionating and washing the fractions, I preferably wash the light oil and fractionate the so purified article. Subsequent washing of the so separated benzol, toluol, and xylols is not requisite. 70 But it is with the residue that I have to do.

I treat the light oil with sulphuric acid in usual manner, then neutralize in usual manner, and then fractionate. The residue is principally coumarone, with some naphthalene, some high-boiling point oils, some sulphonated products. The ingredients are 75 essentially the same as those found in the residues derived from the usual practice as outlined above though the proportions are somewhat different, with consequences which presently I shall indicate.

To this residue I add water (10%) and then a petroleum oil of specific gravity from .8 to .9. Preferably the oil which I here 80 add is such oil as is used for the initial absorption, having specific gravity of from .83 to .86. I add this to the amount of 20%. I bring the whole to a temperature of 80° C. and then allow it to cool and stand for 85 48 hours. An emulsion is produced, and by standing a gravitational separation takes place. The lighter oil above is decanted off, and a semi-solid mass remains.

This remaining semi-solid mass is heated, 90 and, because of the presence of water within and forming part of the emulsion, a steam distillation ensues. The heating is continued until the water is entirely driven off and a temperature of 180°-200° C. attained. The heat is then shut off and the oil which before the immediately preceding steam distillation had been decanted off is now returned, in quantity sufficient to give 95 a finished product of proper consistency for the intended purpose. This quantity will be greater or less, depending upon the variable condition of viscosity which in practice exists, and according to the desired viscosity of the ultimate product. Ordin-

95

100

105

110

narily, the amount of oil so returned will be 10%, more or less, of the total volume.

When the oil has been so returned to the mass the whole is allowed to stand for about 5 five days, during which period a coagulation takes place.

Thus I may obtain a mobile oil which is essentially coumarone, having a specific gravity of about .88, a flash point of about 10 115° C., and a fire point of about 125° C. This product I find to be an excellent cutting oil, that is to say an oil used to flush to cool and to lubricate the operation of cutting steel and like material under a steel tool. As a cutting oil, it is as good as the best, and is derived, as I now have made plain from a by-product commonly regarded as valueless and an annoyance, to make disposal of.

20 Manifestly the oil is useful generally where oils of its viscosity and associated physical properties are useful. And, as I have intimated, its viscosity and allied properties may be varied, by varying the proportions in which the ultimate composition of ingredients is made.

I have said that I prefer, having produced light oil to wash before fractionation. I have explained, however, that the usual way 30 to proceed is to fractionate the light oil, then wash the fractions, and then distill again. And I have explained that if this be done there will remain after such distillations, residues which are still essentially coumarone 35 compounds, with small associated quantities of other substances, such as I have named.

I may so proceed and so obtain my coumarone residue, and in case I do so, I proceed with it, in like manner as I proceed with 40 the coumarone residue of my preferred procedure, the only difference being that in the case I here am considering it is necessary in order to produce an oil of like consistency to add to the coumarone residue petroleum oil of .8 to .9 specific gravity in larger 45 measure than 20%.

In a companion application filed by me on even date herewith, Serial No. 634,605, I have described and claimed a method and the 50 product thereof, which in large part is identical with the method herein described,

but specifically distinct from the invention herein claimed.

I claim as my invention:

1. The method herein described of deriving a by-product oil from the residue which remains after treating the light oil derived from coke-oven gas with sulphuric acid, for the separation therefrom of benzol, toluol, and the xylols, such method consisting in 60 adding to such residue petroleum oil and water, heating, then cooling, and allowing the mass to stand, then decanting off the lighter oil, subjecting the remaining semi-solid mass to distillation, then adding oil 65 to the residue, and allowing the mixture to coagulate.

2. The method herein described of deriving a by-product oil from the residue which remains after treating the light oil derived 70 from coke-oven gas with sulphuric acid, for the separation therefrom of benzol, toluol, and the xylols, such method consisting in adding to such residue petroleum oil and water, heating, then cooling, and allowing 75 the mass to stand, then decanting off the lighter oil, subjecting the remaining semi-solid mass to distillation, returning to the mass previously decanted lighter oil, and allowing the resultant mass so compounded 80 to coagulate.

3. The herein described method of treating a residue containing coumarone which consists in adding to it petroleum oil and water, heating, allowing the mass to cool and settle, decanting, subjecting the remaining semi-solid mass to distillation, then adding oil, and allowing coagulation to follow. 85

4. The method herein described of treating a residue containing coumarone which 90 consists in adding to it petroleum oil and water, heating, allowing the mass to cool and settle, decanting off the lighter oil, subjecting the heavier mass to distillation, returning to the residue previously decanted lighter oil, and allowing coagulation to follow. 95

In testimony whereof I have hereunto set my hand.

FRED W. WAGNER.

Witnesses:

JOHN NUTTALL,  
ROBERT C. KEOGH.